

1

2,866,707

MAGNESIUM HYDROXIDE SIZED  
PHOTORESITIVE PAPER

Hugo H. Hanson, Wynneswood, Pa., assignor to W. C. Hamilton & Sons, Miquon, Pa., a corporation of Pennsylvania

No Drawing. Application February 1, 1955  
Serial No. 485,623

7 Claims. (Cl. 96—75)

This invention relates generally to the manufacture of blueprint paper and more particularly to improvements in the composition thereof and in the method of producing the same.

Heretofore and prior to the present invention, considerable attention has been devoted to the problem of producing a blueprint paper which, when developed, afforded maximum contrast between the blue background and the white lines of the developed print. The usual practice in the art has been to coat the base paper with a light sensitive coating, precipitated from iron salt solutions, which functioned, when exposed to light under an original drawing, washed to remove the chemicals not affected by the light, then developed in a suitable developing solution, such as potassium dichromate and finally dried, to produce a negative wherein the design of the original drawing showed up white against a blue background.

Various attempts have been made to increase the intensity of the blue background of the print, as by improving the composition of the paper base and/or the light sensitive coating, as well as the method of applying said coating. It has been proposed also to precoat the paper base prior to application of the light sensitive coating in order to impart to the fibers of the paper surface an increased capacity to absorb and retain the light sensitive solution which is later applied to the paper. This precoating treatment is necessarily applied to the base paper by coaters who specialize in such processing of the paper base and, of course, adds materially to the cost of the blueprint paper so processed.

I have found that blueprint paper produced in accordance with my present invention, when coated with a suitable light-sensitizing solution, produces prints having a background of a uniformly intense pure blue color against which the design of the original drawing is sharply delineated in white, the contrast between the deep blue background and the white lines of the developed print being exceedingly sharp. Because of the fact that the improved blueprint paper of the present invention provides a print wherein the blue color of its background is of materially increased intensity, the printing time required for producing a satisfactory print of a given drawing may be reduced considerably.

In the preparation of the blueprint paper of the present invention, the paper stock in the form of a conventional suspension or slurry of finely divided rag and/or wood pulp having incorporated therein a suitable internal sizing of rosin and aluminum sulphate is conventionally fed over a wire screen conveyor from which it emerges as a paper web of continuous length, this web being then passed successively through suitable pressing rolls and drying cylinders to a surface sizing station wherein the dried web of paper is surface coated with the sizing solution of the present invention. Thereafter, also in accordance with conventional paper making procedure, the surface-sized paper is calendered and then wound into rolls of any desired size, in which form the paper is supplied to the

2

blueprint coaters in condition ready to be surface coated with the requisite light-sensitizing solution.

The solution for surface-sizing the paper in accordance with the present invention includes as its principal ingredient finely precipitated magnesium hydroxide, which, when deposited out of the sizing solution onto the surface of the paper, not only so increases the area thereof that a greater than normal amount of the light sensitizing solution may be applied to the paper, but also increases the wetability of the paper surface for its better absorption and retention of the light sensitizing coating.

Photomicrographic studies of ordinary blueprint paper base coated with light sensitizing solution indicate that this coating solution stains the paper base only to a depth of approximately one fiber diameter, in consequence of which the coating is apt to appear speckled under the microscope.

From photomicrographic study and analysis of the blueprint paper processed in accordance with the present invention it was noted that in such paper, when surface coated with the light sensitive solution and then exposed to light and developed pursuant to conventional blueprinting procedure, the blue pigment of the finished print, consisting primarily of Prussian blue, penetrated the paper to a depth of at least two fiber diameters and that all of the fibers at the coated surface of the paper were uniformly stained blue throughout their cross-sectional areas, thus indicating exceedingly good penetration and retention of the light sensitive solution in the paper surface. It was noted also that in the paper processed in accordance with the present invention, the after-applied light sensitive coating was much more uniformly distributed throughout the paper surface, so much so, that upon exposure and development of the paper, there was obtained a much more even dispersion and deposition of the blue pigment about and between the fibers of the paper immediately adjacent the surface thereof, resulting in a blue background which was free of any appreciable speckling such as causes the appearance of an objectionable slate blue color.

The surface sizing solution of the present invention is prepared in accordance with the following preferred formula:

|                                  |         |     |
|----------------------------------|---------|-----|
| Water                            | gallons | 500 |
| Magnesium hydroxide              | pounds  | 120 |
| Glue                             | do      | 75  |
| Formaldehyde (20% concentration) | gallons | 1   |

The magnesium hydroxide employed in the sizing solution is of microscopic particle size and in all material respects, is the same as that conventionally prepared for medicinal purposes, e. g., as an antacid in milk of magnesia, while the glue of the composition may be any form of animal, vegetable or other glue of good quality, preferably such as is manufactured from proteinaceous material of animal or vegetable origin. In the above formula the magnesium hydroxide represents about 2.7 percent of the weight of the solution, but it will be understood that this percentage may vary within a range of from 1 to 7 percent. Also, the proportions of the glue and of the formaldehyde as respectively set forth in the above example may vary plus or minus 10 percent.

In certain cases it may be desirable to employ hydrated magnesium hydroxide in the form of a paste, in which event a sufficient amount of the paste would be used to include the magnesium hydroxide in a solution in an amount ranging from 1 to 7 percent by weight of the solution.

The magnesium hydroxide, which is difficultly soluble, is present in the solution as a water dispersion, in which form it is maintained by the glue content of the solution. On passing the paper web through this surface sizing solu-

tion, there is deposited on the paper a surface layer of discrete microscopic particles of the magnesium hydroxide. The magnesium hydroxide particles are permanently fixed to the surface by the glue contents of the solution, the glue itself being tanned or hardened by the formaldehyde to better condition the paper surface against being adversely affected by the wet processing treatments to which it is subsequently subjected, e. g., the application of the light sensitizing solution and the conventional blueprinting steps.

In lieu of employing formaldehyde to tan or harden the glue in the composition of the formula above set forth, there may be employed melamine, urea formaldehyde, hexamethylene tetramine or aluminum sulphate. It will be understood, also, that any other suitable binding agent may be employed for fixing the deposited particles of magnesium hydroxide upon the surface of the paper, as for example, suitable vegetable starches or organic derivatives of cellulose, such as carboxy-methyl cellulose and carboxy-ethyl cellulose. In any event, the binding agent, whether it be one consisting of glue combined with a hardening agent, e. g., formaldehyde or any of its above mentioned substitutes, or one which does not include glue as a constituent, e. g., vegetable starch, carboxy-methyl cellulose, or carboxy-ethyl cellulose, is present in the composition in an amount sufficient to permanently fix on the sized surface of the paper a layer of uniformly distributed microscopic particles of magnesium hydroxide. As indicated by the above formula, the binding agent is present in the composition in an amount which preferably approximates 50 to 75 percent of the weight of the magnesium hydroxide in a water dispersion thereof.

It is believed that the improved background color, contrast of the white lines with the background color and speed of printing of the blueprint paper prepared in accordance with the present invention result not only from the fact that the layer of microscopic particles of magnesium hydroxide on the surface of the paper increases the area, depth and concentration of the light sensitizing coating subsequently applied to the paper, but also from the fact that the magnesium hydroxide sizing solution is of a pH of from 8.5 to 10 and thus is of an alkalinity sufficiently high to weaken the internal sizing slightly and insure penetration of the light sensitizing solution into the surface of the paper for a depth of at least 2 fiber diameters, in consequence of which the light sensitizing solution at the surface of the paper is in substantially continuous phase.

Inasmuch as magnesium hydroxide is quite stable at the normal operating temperature of the surface sizing solution, which temperature is from 125 to 140° F., as determined by the heat of the paper delivered from the drying rolls to the surface sizing bath, it will be apparent

that the surface sizing solution of the present invention may be advantageously applied to the paper by the ordinary tub sizing procedure such as is now conventionally used in paper making mills for the preparation of blueprint paper.

It will be understood, of course, that the present invention is susceptible of various changes and modifications which may be made from time to time without departing from the general principles or real spirit thereof, and it is accordingly intended to claim the same broadly, as well as specifically, as indicated by the appended claims.

What is claimed as new and useful is:

1. A photosensitive paper comprising a paper base having thereon a surface sizing of magnesium hydroxide and an agent for fixing the magnesium hydroxide upon the paper surface, and a light sensitive coating on said sized paper base of light sensitive salts.
2. A photosensitive paper as set forth in claim 1, wherein said agent is glue.
3. A photosensitive paper as set forth in claim 1, wherein said agent is the reaction product of a glue derived from proteinaceous material and formaldehyde.
4. A photosensitive paper as set forth in claim 1, wherein said agent is glue combined with a glue hardening agent selected from the group consisting of formaldehyde, urea formaldehyde, melamine, aluminum sulfate, and hexamethylene tetramine.
5. A photosensitive paper as set forth in claim 1, wherein said agent is a vegetable starch.
6. A photosensitive paper as set forth in claim 1, wherein said agent is an organic derivative of cellulose.
7. A photosensitive blueprint paper comprising a paper base having thereon a surface sizing of magnesium hydroxide and an agent for fixing the magnesium hydroxide upon the paper surface, and a light sensitive blueprint coating on said sized paper base precipitated from an iron salt solution.

#### 40 References Cited in the file of this patent

#### UNITED STATES PATENTS

|           |              |               |
|-----------|--------------|---------------|
| 51,010    | Brinckerhoff | Nov. 21, 1865 |
| 61,338    | Hoover       | Jan. 22, 1867 |
| 1,934,639 | Rafton       | Nov. 7, 1933  |
| 1,935,434 | Cohen        | Nov. 14, 1933 |
| 2,608,546 | Jackson      | Aug. 26, 1952 |
| 2,626,867 | Webster      | Jan. 27, 1953 |
| 2,639,989 | Conover      | May 26, 1953  |
| 2,705,685 | Cipriano     | Apr. 5, 1955  |

#### 45 OTHER REFERENCES

Institute of Paper Chemistry, Clarence J. West, Bibliographic Series, Number 165. Copyright 1945, Sizing of Paper.